

March 13, 1945.

E. CZAPEK

2,371,155

MACHINE AND PROCESS FOR MAKING CELLULOSE FILMS AND THE LIKE

Filed Aug. 3, 1940

2 Sheets-Sheet 1



INVENTOR  
EMIL CZAPEK  
BY *Gustav Drews*  
ATTORNEY

March 13, 1945.

E. CZAPEK

2,371,155

MACHINE AND PROCESS FOR MAKING CELLULOSE FILMS AND THE LIKE

Filed Aug. 3, 1940

2 Sheets-Sheet 2



INVENTOR  
EMIL CZAPEK  
BY  
Gustav Drews  
ATTORNEY

## UNITED STATES PATENT OFFICE

2,371,155

## MACHINE AND PROCESS FOR MAKING CELULOSE FILMS AND THE LIKE

Emil Czapek, New York, N. Y.

Application August 3, 1940, Serial No. 350,291  
In Germany December 17, 1935

7 Claims. (Cl. 18—15)

This invention relates to a process for, and to an apparatus for carrying out the process of, the manufacture of films, foils, membranes, bands, sheets and the like from solutions of cuprammonium cellulose. This application is a continuation in part of my co-pending application, Serial No. 116,290, filed December 17, 1936.

This invention has for an object the manufacture of foils, films, pellicles and the like by pouring a cuprammonium cellulose solution onto a movable support, especially onto a molding belt, and coagulating and solidifying the poured solution, and thereafter continuing the further treatments, mainly the regeneration of the cellulose on said support without detaching the resulting film strip from the support until the chemical conversion, purification and the like are completed, so that after the detachment practically only washing and drying of the film are still necessary.

These and other features, capabilities and advantages of the invention will appear from the subjoined detail description of specific embodiments illustrative of apparatus for carrying out the processes of the invention illustrated in the accompanying drawings, in which

Figures 1 to 6 inclusive illustrate diagrammatically and by way of example various embodiments of the apparatus in side elevation; and

Fig. 7 is a diagrammatic sketch illustrative of the progress of drying of the cellulose pellicles.

As aforesaid, the present invention has for an object the manufacture of foils, films, pellicles and the like by the so-called "wet" process while using a support for the treatments of the film strip as long as possible.

In the so-called "dry" process, the advantage of working on a movable support as long as possible, has been recognized for a long time. In such cases the working operation is invariably the same, that is, a viscous solution of a cellulose ester in organic volatile solvents is poured onto the pouring belt and solidifies during the travel of the belt in its path of movement due to the gradual evaporation of the solvents. Shortly before the belt returns to the pouring device, the applied coating is dried, so that it can be detached from the support in the solid condition.

The "dry" casting process there requires only the application of heat and effluent air for the removal of the solvent vapour, so that the utilisation of the support until the finished film is detached would appear to be more or less compulsory from the outset.

On the other hand, this method of working has not been adopted for the "wet" process, according to which a viscous cellulose solution is caused to precipitate by several wet agents such as water, saline solutions, acids and alkalies, for the purpose of forming a film. Since the cellulose solution must be brought into contact with a liquid for the purpose of coagulation, and every further phase of the treatment requires renewed contact of the coating with various other liquids, the support in the "wet" process, if at all was used for the coagulation only, and the film structure was detached from the support as soon as formed.

15 The value of said support in the further stages of the process was thus lost, and the film formed had to be passed, freely suspended and supported at a few points by rollers and feed cylinders, through a large number of treatment baths. In such a process the film is exposed to all mechanical influences which may give rise to breakage, folding up, and the like. In addition the tension, caused by motion of the machine, would effect an elongation in the longitudinal direction, 20 whereby of course a shrinkage in the transverse direction necessarily follows. This shrinking in the transverse direction in turn would cause the original film to shrink to a greater extent in the transverse direction than in the longitudinal direction, and thus, despite the pouring out of very wide film layers and accordingly wide molding devices, the finished product would turn out in the end to be a relatively narrow film.

The present invention also avoids all these drawbacks, attendant on the one hand on freely suspended lengths of film, and on the other hand on premature detachment of the still unconsolidated film, by utilizing the pouring support until the film has been passed through all the necessary chemical treatment phases.

In order more clearly to understand the invention, reference is made to the accompanying drawings, which illustrate diagrammatically and by way of example, in Figs. 1 to 6, various embodiments thereof.

In said drawings, the following are denoted: the pouring device 1, the pouring belt 2, the guide drums 3, 4, 5, 6 and 7, the spraying devices 8 and 9, the receptacles 10 for coagulation liquid, 35 a detaching or stripping roller 11, a transferring roller 12 for the treatment liquid, couch roller or rollers 13 for draining of the treatment liquid, a transferring belt 14, the detachment at 40 15 of the solid film strip from the support, the

arrows 16 and 17 to indicate the direction of movement of the pouring belt.

In the embodiment shown in Fig. 4, provision is made for enclosing the bath container and for exhausting and recovering the evolved vapours through pipe 18 and fan 19.

The invention will now be described with reference to the following example:

A solution of cuprammonium cellulose containing approximately seven per cent of cellulose and five percent of ammonia, is spread out by means of a slot feeder 1 or other suitable spreading device, see Fig. 1, on an endless molding belt 2. The belt moves by rotation of the drums 3, 4 and 5 in the direction of the arrows 16 and 17. The spread out cellulose solution, by travelling with the moving belts, reaches the downwardly disposed part of the path of movement between the drums 3 and 4, where the cellulose solution is first wetted with a coagulation liquid consisting of a six per cent aqueous caustic soda solution initially to coagulate the solution, and subsequently wetted with water or with a similar alkaline solution but preferably of a lower concentration effectively to solidify the solution. The wetting operation is effected in Fig. 1 by spraying the coagulation liquid onto the cellulose solution by means of a spraying device 8, although the application can also be effected otherwise, for instance by means of applying rollers 12, as illustrated as an instance in Figs. 3 and 6, wetted with the desired liquid. Excess of this liquid is received in the receptacle 10, see Fig. 1, or is removed by means of couch rollers 13, see Figs. 2 and 6.

The direction of motion of the supporting belt changes at the drum 4, see Fig. 1. The cellulose solution is thus now coagulated on the belt. Shortly afterwards, and during its passage through the zone between the drums 4 and 5, the film structure previously coagulated and thereby transformed into a film, is treated with a four per cent aqueous solution of sulphuric acid by means of which said film structure is decopperized and regenerated into cellulose hydrate. The regeneration liquid may be also brought into contact with the film structure by means of a spraying device 8, as shown in Fig. 1, a spreading device, a transferring roller 12, as shown in Figs. 3 and 6, or a felt belt 14 as shown in Figs. 2 and 5, thoroughly soaked with the regeneration liquid and which roller and belt press against the film structure from the outside.

Thereupon the regenerated and decopperized solid film structure leaves the belt on the detaching or stripping roller 11, as shown in Figs. 1 to 6, to be subjected to further treatments, including rinsing and drying treatment.

After completion of the chemical treatment, the film consisting of regenerated cellulose has already sufficient strength to preclude all fear of breakage in the freely suspended portion during the washing and drying treatment. Moreover, there is no objection in principle to carrying out this last wet phase of treatment on the pouring support also, and in passing the washed film from said support directly to the drying apparatus.

The improved drying process of the present invention proceeds from the fact that the cellulose film, since it is not a porous material, behaves in a manner fundamentally different than that of paper or textile fabric during the drying process. The water present in the interior of the film has no opportunity of evaporating

through any pores or interstices, but must escape during heating through the homogeneous surface of the film structure.

It is known that with cellulose films the surface dries more quickly than the inner layers. Furthermore, the drier that the surface is, the greater is the resistance that it offers to the diffusion of the water included in the interior.

The initial drying process accordingly counteracts the subsequent evaporation of the water present in the interior of the film, which naturally also retards the drying process and also gives rise to undesirable differences in tension between the surface and the inner layers of the film, the result being the known irregularities in shrinking, deformations, creases and stresses in the finished film.

It has now been ascertained in accordance with the present invention that the described difficulties can be avoided and the drying effected more rapidly and economically by conducting the drying process in such a manner as to avoid hardening of the surface by said drying. The present invention achieves this by commencing the drying in a moist atmosphere saturated with water vapour and only reducing the vapour content of this atmosphere as the drying progresses. The warming of the film structure and the moisture contained therein to the necessary evaporating temperature is effected according to the present invention:

(a) By means of drying cylinders, heating supports or similar devices preferably internally heated, and

(b) By means of the hot vaporous atmosphere surrounding the film.

It is essential that the drying temperature of the drying cylinder, and the like on the one hand, and the temperature of the vapour atmosphere on the other hand, should be adjusted in relation to each other and both should be adjusted relatively to the vapour content of the heating atmosphere in such a manner that the foregoing favorable diffusion process may take place.

The present invention therefore provides a process for drying cellulose pellicles and the like, in which the drying process is commenced by heating the wet cellulose structure by means of a heated vapour or heated atmosphere and for a heated drying support for the cellulose structure up to the particular temperature of drying desired, which vapour atmosphere in relation to the film temperature at the time is at least saturated with vapour, and then continuing the drying process, if the film structure is heated to the predetermined drying temperature by gradually allowing the vapour content to fall in accordance with the progress of the drying of the film structure, that is in accordance with the progress of the diffusion of the water vapour from the interior to the surface of the film structure. The drying temperature will during this time remain practically constant.

The surprising result of this process is shown in the diagrammatic sketch, Fig. 7, attached hereto, in which diagram the drying time and the degree of drying out at any time are plotted as ordinate and abscissa respectively. The two curves show the progress of the drying in accordance with the former principle (a) and the principle underlying the invention (b). Whereas in the case of the former drying principle the amount of water evaporated is initially many times larger than that in accordance with the invention, nevertheless in the new method of work-

ing as the curve shows, the drying process is completed considerably earlier than hitherto. The progress of the curve (b), which is almost a straight line, shows how uniform is the drying, and investigation of the thus dried product confirms that it is also free from tension, it does not split when cut, and is more resistant to tearing than the hitherto known products.

The present invention, owing to the resultant economy in heat and shortening of the drying time, unites the advantage of an economical working with that of products of improved quality. The present process can in general be carried out on any machine or apparatus, which enables the pouring support to be passed through the various treatment liquids necessary for the formation of the film, or to allow said liquids to act in a suitable manner on the film engaging, and forming on, said support for example by spraying.

The ordinarily used type of belt pouring machine, such as is used for the manufacture of acetate foils and photographic films by the "dry" method, cannot be used for the "wet" process of the present invention owing to the necessity for treating the film with several wet reagents, as mentioned above. These belt pouring machines with two guiding drums for the pouring belt have not hitherto been used in practice for the wet process, because it is not easy to solve the problem of installing the drums and the lower half of the pouring belt with respect to the usual construction of the apparatus. Moreover, the flat elongated shape of the aforesaid apparatus is not favourable for running a belt with a film coating thereon through a precipitating bath because the film lies at the underside and can therefore readily peel off or fall off from the support of its own accord. A film coating so loosened or peeled off from the support gives rise to producing the same troubles as accompany an unsupported film, and which also are difficult to avoid on account of the principle of the aforesaid pouring machine type.

A belt pouring machine, however, can therefore be used for this process, according to the present invention. Such machine fulfills the requirements, to-wit, that the poured cellulose solution coming into contact with the treating liquids must not run off the belt and, when it subsequently solidifies, that the resulting film structure should not become detached from the belt prematurely. To this end and in accordance with said requirements, the apparatus of the present invention comprises not two guide drums for the belt as hitherto customary, but three or more guide drums some of which, generally two, are mounted outside of the liquid, while the others are accommodated completely or partially within the liquid. The belt therefore does not run in two horizontal, antiparallel paths of movement as is the case with ordinary belt machines, but in a triangular or rectangular path of movement. By this means, it is possible for the greater part of the belt to be immersed in the liquid, since the upper "dry" portion, which serves for the pouring, can be made as short as desired by placing the two upper drums correspondingly close to each other. On the other hand, the "wet" portion can be made as long as is required for the chemical process by the suitable location of the third or also of a fourth or fifth drum.

In accordance therewith, the pouring slit is located over the upper or "dry" run of the pouring belt, while the belt itself is guided in an in-

clined direction for the first portion at least and for the major portion of its travel through the precipitating baths.

This arrangement also affords the advantage that the film precipitated on the surface of the belt does not sag downwards in a long horizontal stretch, but receives better support on the drums. It therefore does not possess any tendency to detach itself from the support or to tear owing to its dead-weight, but lies against the belt. Moreover this arrangement permits a compact and compendious construction particularly in belts of 50 and 100 yards in length. Finally it is possible with this arrangement to enclose the liquid container in a simple and ingenious manner so that it is possible to exhaust and recover the vapours.

The pouring belt and/or the drums may be heated or cooled in a manner known per se. For the supporting belt and the drums also non-corrosive kinds of steel are preferably employed, or the supporting belt and the drums are protected from the varying actions of the treatment baths by means of non-corrosive coatings.

In accordance with this invention, the drying may be carried out in practice with any drying machine suitable for drying this product, improved by modifications of individual parts and by supplementary mechanical devices. For example, a cylinder drying machine heated with steam, hot water, oil, and the like, is supplemented by a system of pipes through which there is blown onto or between each pair of the several cylinders, air at the appropriate temperature, and of the requisite water vapour content, or else the drying machine is enclosed in surrounding walls in the manner customary in these drying machines. Partition walls are disposed at suitable places inside the surrounding walls which enable different vapour contents of the surrounding atmosphere to be maintained. The necessary adjustment, regulation and maintenance of this vapour atmosphere is effected on the one hand, by supplying varying quantities of dry air to the separate chambers, and on the other hand, by conducting away varying quantities of the vapours evolved during drying.

It is obvious that various changes and modifications may be made to the details of construction without departing from the general spirit of the invention as set forth in the appended claims.

What I claim is:

1. The process of manufacturing films, foils, membranes, bands and the like, from a cuprammonium cellulose solution while continuously supported during coagulation and regeneration, which comprises pouring the cellulose solution on the outer face of an endless movable support to form a layer, coagulating the layer by a coagulating liquid while still on the outer face of the support, thereupon regenerating the layer so coagulated by a regenerating liquid while still on the outer face of the support, and only then removing the layer so regenerated from the initial support to prevent any interruption in supporting the layer before being finally removed.

2. The process of manufacturing films, foils, membranes, bands and the like, from a cuprammonium cellulose solution while continuously supported during coagulation and regeneration, which comprises pouring the cellulose solution on the outer face of an endless movable support to form a layer, coagulating the layer by a coagulating liquid while still on the outer face of the support, thereupon regenerating the layer

so coagulated by a regenerating liquid while still on the outer face of the support, thereupon washing the layer while still on the outer face of the support, and only then removing the layer from the support and transferring it for a drying treatment.

3. The process of manufacturing films, foils, membranes, bands and the like, from a cuprammonium cellulose solution while continuously supported during coagulation and regeneration, which comprises pouring the cellulose solution on the outer face of an endless movable support to form a layer, coagulating the layer by a coagulating liquid while still on the outer face of the support, thereupon regenerating the layer so coagulated by a regenerating liquid while still on the outer face of the support and then transferring the layer so regenerated from the initial support, the coagulating and regenerating liquids being applied by spraying or the like.

4. The process of manufacturing films, foils, membranes, bands and the like, from a cuprammonium cellulose solution while continuously supported during coagulation and regeneration, which comprises pouring the cellulose solution on the outer face of an endless movable support to form a layer, coagulating the layer by a coagulating liquid while still on the outer face of the support, thereupon regenerating the layer so coagulated by a regenerating liquid while still on the outer face of the support and then transferring the layer so regenerated from the initial support, the coagulating and regenerating liquids being applied by transferring the same onto the layer from wetted transfer rollers or the like.

5. The process of manufacturing films, foils, membranes, bands and the like, from a cuprammonium cellulose solution while continuously supported during coagulation and regeneration, which comprises pouring the cellulose solution

on the outer face of an endless movable support to form a layer, coagulating the layer by a coagulating liquid while still on the outer face of the support, thereupon regenerating the layer

5 so coagulated by a regenerating liquid while still on the outer face of the support and then transferring the layer so regenerated from the initial support, the coagulating and regenerating liquids being applied to the layer by transferring the same from a wetted transfer belt or the like.

6. In an apparatus for the manufacture of extensive lengths of sheets, films and the like, the combination of an endless supporting belt, guiding drums solely on the inside of said endless belt for movably supporting said belt, a pouring device for pouring a cellulose solution on the belt to form a supported layer, means for successively applying treatment liquids including coagulating and regenerating liquids to the supported layer without in any way interrupting its support on said single supporting belt, and means for finally removing the layer so treated.

7. In an apparatus for the manufacture of extensive lengths of sheets, films and the like, the combination of an endless supporting belt and a drying apparatus, guiding drums solely on the inside of said endless belt for movably supporting said belt, a pouring device for pouring a cellulose solution onto the belt to form a supported layer, means for successively applying treatment liquids including coagulating and regenerating liquids to the supported layer without in any way interrupting its support on said single supporting belt, means for washing the layer while still supported on said belt, and means for finally removing the layer from said belt and transferring it to the drying apparatus.

EMIL CZAPEK.